

# United States Patent Office

2,761,801

Patented Sept. 4, 1956

1

2,761,801

## GRAY CAST IRON AND CYLINDER SLEEVE COMPOSED THEREOF

Adna A. Armstrong, Mentor, Ohio, assignor to Thompson Products, Inc., Cleveland, Ohio, a corporation of Ohio

No Drawing. Application October 11, 1952,  
Serial No. 314,409

5 Claims. (Cl. 148—31)

The instant invention relates to an improved method of preparing an article having dimensional stability at high temperatures, and the article resulting therefrom, and more particularly to an improved automotive cylinder sleeve of gray cast iron, and the improved composition thereof and the improved method of making the same.

Articles which are inexpensive to prepare and which have the structural strength of cast iron are in great demand in industry for a number of different purposes, and particularly there is a demand for such articles having dimensional stability at high temperatures. For example, in connection with the particular problem with which the instant invention is principally concerned, namely, the provision of suitable automotive cylinder sleeves, there is a very great need for the provision of such cylinder sleeves that have suitable dimensional stability at the high operating temperatures obtained in the combustion zone in combustion engines such as the diesel engine. It has been found that the cast iron cylinder sleeves heretofore used in certain diesel engines had a tendency to shrink diametrically after a certain period of operation. As will be appreciated, this shrinkage or sleeve collapse results in increased wear of the sleeve by the ring assembly, and no doubt also results in further overheating of the sleeve by virtue of inefficient heat transfer from the sleeve to the block. This collapse problem greatly complicated the problem of providing suitable cast iron cylinder sleeves, which otherwise possess a great number of superior and industrially advantageous properties.

Elaborate studies of this problem have revealed certain differences in collapse properties resulting from casting the iron by different methods, such as sand casting as contrasted to centrifugal casting. Different methods of hardening and tempering or drawing were also investigated; but it appeared that, prior to the instant invention, no one had been able to reach a satisfactory solution to this problem.

The instant invention is based upon the discovery that, by suitable adjustment of the alloying ingredients or additives in a unique manner in cast iron, it is possible to obtain sleeves or the like articles having the properties desired, using industrially acceptable casting, hardening and drawing operations.

It is, therefore, an important object of the instant invention to provide an improved article, cylinder sleeve or the like having dimensional stability at high operating temperatures, and to provide an improved composition for and method of preparing such article.

It is a further object of the instant invention to provide an improved method of preparing an article having dimensional stability at high temperatures that comprises melting and then casting a composition of  $4\pm0.4\%$  silicon,  $2\pm0.3\%$  chromium,  $3.25\pm0.25\%$  total carbon,  $0.8\pm0.2\%$  combined carbon, and the remainder iron and incidental impurities.

It is another object of the instant invention to provide

2

an improved automotive cylinder sleeve composed of gray cast iron having substantially the composition:  $3\frac{1}{2}\text{--}5\%$  silicon,  $1\frac{1}{2}\text{--}2\frac{1}{2}\%$  chromium, the remainder iron and incidental impurities.

5 It is still a further object of the instant invention to provide an improved method of preparing automotive cylinder sleeves, that comprises casting to substantially the desired sleeve shape and size a gray cast iron having  $3\frac{1}{2}\text{--}5\%$  silicon,  $1\frac{1}{2}\text{--}2\frac{1}{2}\%$  chromium, the remainder iron and incidental impurities.

10 It is still another object of the instant invention to provide an improved gray cast iron having substantially the composition:  $4\pm0.4\%$  silicon,  $2\pm0.3\%$  chromium,  $3.25\pm0.25\%$  total carbon,  $0.8\pm0.2\%$  combined carbon, and the remainder iron and incidental impurities.

15 Other and further objects, features and advantages of the present invention will become apparent to those skilled in the art from the following detailed disclosure of preferred embodiments thereof.

20 The instant invention consists in, as the most important article embodying the instant invention, an automotive cylinder sleeve composed of gray cast iron having substantially the composition:  $3\frac{1}{2}\text{--}5\%$  silicon,  $1\frac{1}{2}\text{--}2\frac{1}{2}\%$  chromium, the remainder iron and incidental impurities.

25 The essence of the instant invention is that the instant  $2\%$  Cr— $4\%$  Si gray cast iron has unique dimensional stability under the operating conditions ordinarily subjected to automotive cylinder sleeves. As indicated, the amount of silicon employed may range from about  $3\frac{1}{2}$  to about 5 weight percent, and is preferably about 4 weight percent plus or minus 10% thereof, or  $4\pm0.4\%$ . (As used herein, the terms "parts," "percent" and "%" mean parts and percent by weight, unless otherwise specified.)

30 The amount of chromium present in the composition may range from about  $1\frac{1}{2}\%$  to about  $2\frac{1}{2}\%$ , and is preferably  $2\pm0.3\%$ . Heretofore, in the cast irons employed in the production of cylinder sleeves, the amount of chromium employed, if any, was a relatively small amount being less than about 0.5% in all instances. In some steel compositions, however, substantially greater proportions of chromium have been used for one purpose or another in the so-called high chromium steels, but those skilled in the art will readily recognize that the use of steel generally in connection with cylinder sleeves or the like articles involves an entirely different set of problems, and the effectiveness or lack of effectiveness of the use of chromium in a given amount in steel has no relation to the problems here involved in connection with the use of cast iron. As far as the skilled workers in the art were concerned, there was apparently no particular reason for employing more than the relatively minor amounts of chromium heretofore employed in cast irons adapted to this specific use.

35 The instant invention, however, resides not only in the unobvious discovery that substantially increasing the chromium content up to about 2% causes a materially significant change in the cast iron properties, but also that the combination of the high chromium content plus approximately twice as great a silicon content results in a uniquely superior composition for the purposes of the instant invention.

40 As a rule, silicon (as contrasted to chromium) is present essentially as an impurity in small amounts in all cast irons. Ordinary cast iron seldom contains less than about 0.50% silicon, and on some occasions may contain as much as 3% silicon. As it is generally understood, the silicon probably combines with the iron to form the silicide of iron, which is then dissolved in the balance of the iron. Those skilled in the art have recognized that the influence of silicon on the properties of cast iron is very important, chiefly through its known

45 50 55 60 65 70

property of promoting the formation of graphitic carbon, and thereby increasing the softness, and if carried too far, decreasing the strength of the cast iron. Foundry men often speak of silicon as a "softener." Silicon is also understood to influence the decomposition of iron carbide, and the presence of some silicon in the carbide tends to render it less stable. For these, and other reasons, those skilled in the art have in most cases attempted to keep the silicon contents at a minimum, and in the preparation of cast iron cylinder sleeves heretofore a silicon content appreciably in excess of 3% was not used, and it was apparently the general attitude that silicon contents in excess thereof should not be used.

It also appears that the general practice in chromium-silicon steel manufacture involved the use of chromium in amounts of two or more times the silicon content.

The instant invention, however, is based upon the discovery that uniquely superior cast iron cylinder sleeves may be obtained by the use of a composition having a chromium content substantially in excess of that ordinarily used in cast iron adapted to this purpose, a silicon content substantially in excess of that ordinarily used in cast iron adapted to the instant uses, and a silicon content of twice the chromium content, which is substantially the reverse of the chromium-silicon proportions heretofore used in cast irons used for cylinder sleeve manufacture (and is also substantially the reverse of the chromium-silicon proportions used generally in ferrous materials).

Although it is not desired to limit the instant invention to any particular theory or explanation for the superior results obtained hereby, it is believed that there must be some unusual cooperation between the chromium and the silicon so that, among other things, a suitable graphite flake deposition is accomplished so that a unique combination of high wear and abrasion resistance and high dimensional stability under operating conditions may be obtained.

As previously mentioned the instant ferrous material is gray cast iron, which is the name by which cast irons containing a considerable amount of the graphitic carbon are known because of the appearance of their fracture, which is grayish or blackish and coarsely crystalline. In general, such cast irons may contain from 2½ to about 4% carbon, as total carbon content, and in the case of the instant invention the carbon content is preferably  $3.25 \pm 0.25\%$ . The instant cast iron consists of type A graphite, size 4-6, in a matrix that is pearlitic generally in the "as cast" form. The primary carbide content is approximately 4-6%. As will be explained hereinafter, suitable hardening and drawing thereof results in changing the matrix to essentially a tempered martensitic matrix.

As mentioned, in the preferred gray cast iron of the instant invention, the total carbon content is about 3%, plus or minus  $\frac{1}{4}\%$ , and the combined carbon content is about 0.8%, plus or minus 0.2%. The remainder of the composition consists of iron and the incidental impurities ordinarily present in cast iron.

One of the impurities ordinarily present in cast iron is sulfur, which may be present from mere traces (substantially 0%) to about about 0.1%. Sulfur in excess of the stated maximum amount imparts undesirable properties to the cast iron, and in the practice of the instant invention the sulfur content may be about 0-0.1%.

Another impurity ordinarily present in cast iron is phosphorus. Phosphorus may be present in substantially trace amounts (0%) up to about 1.7% in cast irons. In such small amounts, the phosphorus present is understood to form an iron phosphide, which is held in solid solution in the iron. In amounts over about 1.7% the phosphorus develops other functions in the cast iron, and the use of phosphorus in excess of that amount is not desired in the instant invention. Preferably, the phosphorus content is quite low, being less than about 0.5%.

in the cast iron compositions employed in the instant invention.

Still another impurity ordinarily present at least to some extent in cast iron is manganese. Manganese may be present in cast iron in amounts ranging from mere trace amounts to as much as about 2%, and ordinary cast iron usually contains about 0.1-2% manganese. In the instant invention, the amount of manganese present may be about 0-2%, but in some instances it has been found preferable to employ manganese in amounts of about 0.5-1%, since such relatively small amounts of manganese may tend to impart a slight amount of additional hardness to the iron.

Other impurities or additives, such as nickel and copper may also be present in small amounts (i. e., 0.5% or less) in the cast iron of the instant invention.

As an example of the superior results obtained in the practice of the instant invention, cast iron sleeves were made using the compositions 1 and 2 shown in the table below:

#### Composition

|    |                                        | (1)    | (2)    |
|----|----------------------------------------|--------|--------|
| 25 | Total C.....percent                    | 3.40   | 3.26   |
|    | Combined C.....do                      | 0.97   | 0.80   |
|    | Si.....do                              | 3.72   | 1.95   |
|    | Cr.....do                              | 1.78   | 0.34   |
|    | S.....do                               | 0.08   | 0.085  |
|    | P.....do                               | 0.21   | .10    |
| 30 | Mn.....do                              | 0.75   | .66    |
|    | Collapse (1 hr. at 600° F.).....inches | 0.0016 | 0.0025 |

The compositions shown in the above table were sand cast in the form of sleeves, and the general character of the resulting cast metallurgical structure obtained in each case was that it contained type A, size 4 graphite flakes in a pearlitic matrix. In the case of composition 1, which embodies the instant invention, the matrix also contained about 6% of primary carbides. The sleeves were hardened by heating to 1550° F. and quenching, so as to obtain an essentially martensitic matrix, and a hardness of about 48-50. The sleeves were then drawn or tempered, by holding at 600° F. for one hour. In the collapse test, the sleeves are maintained for one hour in an oven at 600° F., and the decrease in diameter thereof (which is about a five inch diameter) which takes place during the heat test is measured. As will be seen in the instant test, the collapse was .0016 inch for composition 1 and .0025 inch for composition 2, thereby showing that the collapse was over 50% greater in the case of composition 2, which was a composition heretofore employed in the sand casting of cylinder sleeves in standard practice.

As another demonstration of the superiority of the composition of the instant invention, in this case for purposes of centrifugal casting, compositions 3 and 4, as shown below, were employed in the centrifugal casting of sleeves such as those just described.

#### Composition

|    |                                        | (3)    | (4)    |
|----|----------------------------------------|--------|--------|
| 60 | Total C.....percent                    | 3.18   | 3.42   |
|    | Combined C.....do                      | 0.69   | 1.11   |
|    | Si.....do                              | 3.88   | 2.03   |
|    | Cr.....do                              | 1.88   | 0.43   |
|    | S.....do                               | 0.08   | 0.05   |
|    | P.....do                               | 0.11   | 0.10   |
| 65 | Mn.....do                              | 0.65   | 0.78   |
|    | Ni.....do                              | 0.19   | 0.58   |
|    | Cu.....do                              | 0.24   | 0.52   |
| 70 | Collapse (1 hr. at 600° F.).....inches | 0.0010 | 0.0020 |

The resulting sleeves were hardened and drawn as herebefore described, and again the collapse test results indicate the distinct superiority of composition 3, as contrasted to composition 4 which was a commercially em-

ployed composition for centrifugal casting of cylinder sleeves.

It has also been found that the instant compositions 1 and 3, hereinbefore described, produce cylinder sleeves having superior wear and tear and abrasion resistance and having a much longer operating life during ordinary use.

Again, without limiting the invention to any particular theory, it is believed that the 2% Cr—4% Si gray cast iron has the superior results here shown because of a unique cooperation between the "hardener," chromium, and the "softener," silicon, in these particular proportions, during the casting process. During casting, and particularly sand casting which is preferred for use in the invention, the molten cast iron is poured into the desired shape, and cooling takes place ordinarily at a fairly slow rate so that carbon deposition and flake formation may take place to a sufficient extent to obtain the typical gray cast iron structure.

Unquestionably the instant excessive amount of silicon alone (in the absence of the excessive amount of chromium) would effect such carbon or graphitic flake deposition as to make the gray cast iron too soft and weak. In contrast, chromium is used in steel and as a hardener for tool steel in amounts of less than 1% and in ball bearings in an amount of less than 1½%. (Chromium in the high-chrome steels functions in a different manner metallurgically and is used in amounts of 10, 20 or 30%.) It would appear that the use of chromium in cast iron in amounts in excess of the usual small amount of less than about 0.5% would be wasteful or would result in undue embrittlement of an already brittle material.

Apparently in the instant casting method, however, the chromium in the high amounts used materially interferes with the tendency of the silicon to cause soft graphitic deposits, to the extent that the chromium substantially overcomes this tendency even for the excessive amount of silicon used; or the chromium in the high amount present forms an appreciable percentage of chromium carbides which cooperate with cementite and for graphite per se to impart additional hardness thereto so as to overcome what would be expected to be the harmful softening effects of the excessive silicon. Whatever the peculiar phenomenon involved it seems clear that the cooperative co-action or independent actions of the 2% Cr—4% Si system take place initially during the casting process so as to obtain a suitable "as cast" metallurgical structure.

During subsequent use of this cast material, the chromium and silicon must again cooperate; this time the silicon assisting significantly in the dimensional stability of the article and the chromium probably stabilizing the metallurgical structure to overcome any tendency on the part of the silicon to render the carbides (which would now have high amounts of chromium carbides therein) less stable.

It will be understood that modifications and variations may be effected without departing from the scope of the novel concepts of the present invention.

I claim as my invention:

1. An automotive cylinder sleeve composed of gray cast iron having substantially the composition: 3½—5% silicon, 1½—2½% chromium, the remainder iron and incidental impurities, and having a structure consisting essentially of graphite flakes, and 4—6% primary carbides in a tempered martensitic matrix.

2. A hardened and drawn automotive cylinder sleeve composed of cast iron containing 3½—5% silicon, 1½—2½% chromium, 2½—4% carbon, 0.8±0.2 combined carbon, and the principal part of the remainder iron.

3. An automotive cylinder sleeve cast, and then hardened and drawn to obtain an essentially tempered martensitic matrix, from molten cast iron containing 4±0.4% silicon, 2±0.3% chromium, 3.25±0.25% carbon, 0—0.1% sulfur, 0—1.7% phosphorus, 0—2% manganese and the remainder iron.

4. An automotive cylinder sleeve composed of gray cast iron having substantially the composition: 4±0.4% silicon, 2±0.3% chromium, 3.25±0.25% total carbon, 0.8±0.2% combined carbon, and the remainder iron and incidental impurities.

5. Hardened and drawn gray cast iron having a structure of graphite flakes, 4—6% primary carbides and less than 5% free ferrite in essentially a tempered martensitic matrix, and having substantially the composition: 4±0.4% silicon, 2±0.3% chromium, 3.25±0.25% carbon, 0—0.1% sulfur, 0—1.7% phosphorus, 0—2% manganese and the remainder iron.

#### References Cited in the file of this patent

#### UNITED STATES PATENTS

|           |              |               |
|-----------|--------------|---------------|
| 2,081,304 | Moluf        | May 25, 1937  |
| 2,167,301 | Jones et al. | July 25, 1939 |
| 2,287,850 | Young        | June 30, 1942 |
| 2,518,055 | Olsen et al. | Aug. 8, 1950  |